

## UNITED STATES PATENT OFFICE

JOHN H. MARTIN, OF BALDWIN, NEW YORK

## PREPARATION OF FUR FOR SHRINKING AND FELTING

No Drawing.

Application filed July 14, 1928. Serial No. 292,914.

It is well known that animal fibre which is to be felted, particularly for use in the manufacture of hats, must be subjected to a chemical treatment in order to obtain a satisfactory felted product. Although many substances have been proposed for such preparatory treatment of the fibre, that which has been most generally used heretofore is a solution of nitrate of mercury in nitric acid, which has been found to give results which are satisfactory from the manufacturing point of view, although not from a hygienic standpoint because of its toxic quality. Some other substances, such as sodium peroxide and orthosodium perborate have been proposed and are used to a limited extent although they have been found to be too strongly alkaline.

In the development of the present invention it has been determined that the action of any substance which gives satisfactory results, or nearly satisfactory results, is of a two-fold nature, being hydrolytic and oxidizing in effect on the proteins of the fibre and it has also been determined that the hydrolysis, which depends upon the nature and strength of the acid, time and temperature, should be mild, such as is sufficient to carry the action only to the peptone stage. In the effort to avoid the toxic effect of the nitrate of mercury and at the same time to produce the otherwise satisfactory results due to its use, it has been found, by the present invention, that the desired action upon the fibre is effected by the use of disodium hydrogen phosphate in conjunction with an oxidizing agent, which substances have no known toxic effect. The disodium hydrogen phosphate shows an alkaline reaction but only sufficient to carry hydrolysis to the point desired, while the addition of hydrogen peroxide, both substances being in solution, produces the desired oxidizing effect. Practical tests of these substances with the different furs employed in the manufacture of hats have shown such furs, thus treated, to be equal in felting and shrinking qualities to fur treated with nitrate of mercury, with superior texture and feel.

It will be understood that by reason of the differences between different kinds of animal fibres the proportions of the disodium hydrogen phosphate and the oxidizing agent employed will be varied more or less. It 55 has been found that the amount of disodium hydrogen phosphate can be varied considerably without any appreciable effect, while the amount of available oxygen introduced by the oxidizing agent should be not more 60 than that required by the particular fur to be treated. By way of example, it may be stated that white coney skins can be treated successfully by brushing the fur with a solution containing 30 grams of disodium hydrogen phosphate with 6% of hydrogen peroxide per liter, the skins being worked up in the usual way after drying. As another example, it may be stated that Australian 65 rabbit skins are successfully treated by 70 brushing the fur with a solution containing 60 grams of disodium hydrogen phosphate with 4% of hydrogen peroxide per liter, the skins being worked up in the usual way after drying. 75

It will be further understood that the disodium hydrogen phosphate and the oxidizing agent can be used, in solution, either separately or in mixture.

I claim as my invention:

1. The improvement in the art of preparing fur for shrinking and felting, which consists in subjecting the fur to the action of a solution of disodium hydrogen phosphate and an oxidizing agent.

2. The improvement in the art of preparing fur for shrinking and felting, which consists in subjecting the fur to the action of a mixture of a solution of disodium hydrogen phosphate and a solution of hydrogen peroxide.

This specification signed this 12th day of July A. D. 1928.

JOHN H. MARTIN.